

Aug. 8, 1933.

L. H. BEDFORD

1,921,067

MANUFACTURE OF THERMIONIC DEVICES

Filed Aug. 13, 1929

FIG. 1



FIG. 2



INVENTOR  
L. H. BEDFORD

BY

*Walter C. Kiesel*

ATTORNEY

## UNITED STATES PATENT OFFICE

1,921,067

## MANUFACTURE OF THERMIONIC DEVICES

Leslie Herbert Bedford, Aldwych, London, England, assignor to Western Electric Company, Incorporated, New York, N. Y., a Corporation of New York

Application August 13, 1929, Serial No. 385,698,  
and in Great Britain November 16, 1928

3 Claims. (Cl. 250—27.5)

In the manufacture of various articles of commerce such as thermionic devices, it is frequently necessary to produce an alkaline earth metal vapor inside the article at some stage of manufacture, usually during an evacuation process. For this purpose two methods are well known in the art:

(1) A compound is provided which decomposes on heating to a permanent gas and an alkaline earth metal. Such a compound is barium azide which is said to break down to nitrogen and metallic barium.

(2) A mixture is provided which reacts to form metallic barium. Such a mixture is barium oxide and metallic magnesium which reacts to form metallic barium and magnesium oxide.

Both these methods are in use commercially, but they are both subject to severe limitations. In the first case, barium azide may not decompose completely to the metal, and invariably a certain amount of barium nitride is present. This not only means that a further liberation of nitrogen takes place when the temperature is raised to vaporize the barium, but also sets a limit to the degree of vacuum which can be obtained in the finished article, on account of the vapor or dissociation pressure of the barium nitride which is deposited or formed in various parts of the device. In the second case the gas trouble is theoretically absent, but in practice a great evolution of water vapor accompanies the reaction owing to the impossibility of keeping the barium oxide dry. There is also a more serious objection that a great deal of vaporization of magnesium takes place which inhibits the application of the method in a great many cases.

The present invention provides other sources of barium vapor which are free or more nearly free from the above defects.

According to one feature the present invention provides a source of alkaline earth or rare earth metal vapors for the said purpose in which the metals are provided in a free condition, and provided where necessary with a suitable protection against oxidizing or hydrating. The metals are preferably formed by the action of one or more reducing agents of their compounds, the new compound so formed constituting a protection against oxidation or hydrating. The said protection may be supplemented or effected by a compound such as hydrocarbon or any coating which is conveniently removed by heating in vacuo.

As an example of carrying out the invention

metallic barium may be prepared by a species of thermit reaction. A mixture of barium oxide, barium peroxide, and metallic aluminum is heated, whereupon at a certain temperature (depending principally upon the proportions) a reaction takes place with the formation of metallic barium and aluminum oxide. From this mixture it is comparatively easy to distil the barium in a moderately good vacuum.

The application to the thermionic device may take place at any stage, that is to say either before or after the performance of the thermit reaction, or after the distillation of the barium. Measures may be provided to prevent oxidation or hydration of the source while it is being applied, for instance, to the plate of a valve. Saturated hydrocarbons carefully dried over sodium have been proved suitable as protection, but any other form of protection can be used, such as another metal. Alternatively, it may be preferable to extract the barium from the thermit product, barium and aluminum oxide, by dissolving the barium in another metal.

For example, the finely divided thermit product may be mixed with molten aluminum which takes up the barium in alloy form. A small piece of the resulting alloy serves as the barium source. A similar alloy may also be prepared electrolytically.

In the accompanying drawing, there is shown, in Fig. 1, the envelope 1 of a thermionic or electric discharge device with an anode or plate member 2 and a filament or cathode member 3 therein. The source of thermionically active earth metal vapor in the form of a small pellet 4 may be introduced into the envelope 1 by suitably fastening it to the anode. A source 5 of current external the envelope may be inserted in the cathode circuit by closing the switch 6 and the plate 2 heated by bombardment until the thermionically active earth metal is caused to vaporize. Alternatively, the source of thermionically active earth metal may be heated by high frequency induction currents, the use of which for such purpose being well known. Instead of securing a pellet 4 to the plate as shown in Fig. 1, a recess 7 may be provided in the anode 2 (see Fig. 2) in which the source of thermionically active earth metal may be placed as a paste or in pellet form and covered by a cover plate 8 which permits the egress of the vaporized earth metal when the plate is heated to the necessary degree.

As already indicated, while applying the

source of thermionically active earth metal vapor to the anode of the device, said source may be protected against hydration and oxidation by the use of a protective material, such as saturated hydrocarbons.

What is claimed is:

1. The method of producing a thermionically active earth metal vapor in an envelope of an electric discharge device which consists in introducing into the envelope an alumino-thermic reaction product containing pure thermionically active earth metal and aluminum oxide, and thereafter vaporizing therefrom, the pure thermionically active earth metal.
- 15 2. The method of producing a thermionically active earth metal vapor in an envelope of an

electric discharge device which consists in introducing therein an alumino-thermic reaction product provided with protection against hydration and oxidation, said reaction product containing pure thermionically active earth metal and aluminum oxide, and thereafter vaporizing the pure thermionically active earth metal.

80 3. The method of producing barium vapor in an envelope of an electric discharge device which consists in introducing therein an alumino-thermic reaction product of barium oxide, barium peroxide and aluminum, said product containing metallic barium, and thereafter vaporizing barium from the reaction product.

85

90  
LESLIE HERBERT BEDFORD.

20

95

25

100

30

105

35

110

40

115

45

120

50

125

55

130

60

135

65

140

70

145

75

150